

# United States Patent Office.

HENRY A. LUDWIG, OF NEW YORK, N. Y.

*Letters Patent No. 97,941, dated December 14, 1869.*

## IMPROVEMENT IN THE MANUFACTURE OF ULTRAMARINE.

The Schedule referred to in these Letters Patent and making part of the same.

*To all whom it may concern:*

Be it known that I, HENRY A. LUDWIG, of the city, county, and State of New York, have invented a new and useful Improvement in the Manufacture of Ultramarine, of which the following is a full, clear, and exact description.

My invention consists in a certain mixture or combination of ingredients for the manufacture of artificial ultramarine, whereby an article having a finer color is produced. The proportion of the several ingredients may be more or less varied, as may also the periods of their exposure to heat and the temperature of the ovens in which the mass is treated; also, other ingredients, if necessary, be added, but the ingredients hereinafter named, mixed in or about the proportions described, and treated substantially as specified, I know, from actual experiment, will suffice. As in the treatment of other compounds for the production of ultramarine, I first subject the mass to a high temperature, in one oven, and afterward to a lower temperature, in another oven, for the purpose of desulphurizing it, and prefer to use for such purpose, a furnace in which both ovens, that are arranged one above the other, are heated by the same fire, and which furnace is made the subject of a separate application for Letters Patent.

Thus, discarding the use of sulphate of soda, as generally used in such mixtures, I take, say, eighty to one hundred pounds (80 to 100 lbs.) of carbonate of soda, ninety to one hundred pounds (90 to 100 lbs.) of burnt clay, sixty to one hundred pounds (60 to 100 lbs.) of sulphur, six pounds (6 lbs.) of charcoal, three to four pounds (3 to 4 lbs.) of colophony or rosin, thirty to forty pounds (30 to 40 lbs.) of silicate of potassa or soda, or of both, commonly known as soluble glass, or, in place of this latter ingredient, forty-five pounds (45 lbs.) of silica.

To mix and treat these several ingredients, I take, first, the soda, clay, sulphur, charcoal and rosin, and finely grind the same, and afterward mix them with the soluble glass or silica, and put the mass into the ordinary or any suitable crucibles. These crucibles

are then covered up and placed in the lower or hotter oven of the two ovens hereinbefore referred to, the fire gradually increasing in temperature, until, after from ten to fourteen hours, the mass has been brought to a red heat. After the mass has been in said oven from sixteen to eighteen hours, altogether, this part of the process is completed, and the oven allowed to cool down, and the fused mass taken out and crushed. The mass is then introduced into the upper or cooler oven, and which need only be hot enough to effect desulphurization. It may be placed in iron vessels within this oven, or be spread over the bottom of the same, and may remain in said oven while a fresh charge is being treated in the first oven, so that where the two ovens are combined in the one furnace, the latter need not be opened to interfere with the process going on in the first oven. Upon the mass or color being taken out of the second oven, it is washed, to remove the soda. This may be done in any suitable manner, but I prefer the effect the same by throwing the color into a hogshead fitted with a perforated false bottom, over which coarse linen cloth, previously soaked in water, is spread. The color being put into said hogshead so as to nearly fill it, hot boiling water is poured in until it completely covers the color, which is allowed to remain in soak for about six hours, when the water is drawn off, by means of a faucet near the bottom of the hogshead. Such washing of the color may be repeated twice, after which it is ground and sifted to separate the different grades or qualities, and subsequently dried or roasted in iron pans, and ground again, when it is ready for the market.

Having thus described my improvement in the manufacture of ultramarine,

I claim as new—

The combination of ingredients, herein named, mixed and treated substantially as specified.

HENRY A. LUDWIG.

Witnesses:

F. HAYNES,  
HENRY PALMER.